

# United States Patent Office

3,259,498

Patented July 5, 1966

1

3,259,498

## PHOTOGRAPHIC LAYERS SUITABLE FOR THE SILVER DYESTUFF BLEACHING PROCESS

Walter Anderau, Aesch, Basel-Land, and Helmut Boehl, Bottmingen, Switzerland, assignors to Ciba Limited, Basel, Switzerland, a Swiss company  
No Drawing. Filed May 21, 1962, Ser. No. 196,432  
Claims priority, application Switzerland, May 30, 1961, 6,292/61

9 Claims. (Cl. 96—99)

In the subtractive color photographic process for the production of color transparencies and color pictures to be viewed by reflected light there is required a blue component color image of which the blue dyestuff has an absorption maximum at about 600 to 640  $\text{m}\mu$  and is as transparent as possible in the region from 400 to about 500  $\text{m}\mu$ . When the blue component color image is produced by the known silver dyestuff bleaching process, there are generally used blue azodyestuffs which are bleached in suitable bleaching baths depending on the quantity of image silver locally present.

Various blue azo-dyestuffs are known for use in producing a blue component color image by the silver dyestuff bleaching process. Dyestuffs of this kind also exist among the ordinary commercial direct dyestuffs, for example, the disazo-dyestuffs that are obtained by coupling tetrazotized 3:3'-dimethoxy 4:4'-diamino-1:1'-diphenyl on both sides with 1-amino-8-hydroxynaphthalene-3:6- or -2:4-disulfonic acid. To a large extent these dyestuffs meet the above requirements. However, they have the disadvantage that where the image silver has decomposed the dyestuff to a low color density of about 0.1 to 0.3 logarithmic value a change in shade towards a reddish blue takes place. An explanation of this phenomenon is that the disazo-dyestuffs decompose in stages via the monoazo-dyestuffs as follows:



The present invention is based on the observation that dyestuffs obtained from a tetrazotized 3:6:3':6'-tetraalkoxy-4:4'-diaminodiphenyl and 1-amino-8-hydroxynaphthalene disulfonic acids do not exhibit the above disadvantage in the silver dyestuff bleaching process.

The invention therefore provides photographic layers

2

suitable for the silver dyestuff bleaching process which contain a dyestuff of the general formula



in which  $R_1$  and  $R_2$  each represent the radical of a 1-amino-8-hydroxynaphthalene sulfonic acid bound to the azo linkage in a position vicinal to the hydroxyl group, and at least one of the said radicals contains two sulfonic acid groups, and in which  $X_1$  and  $X_2$  represent an alkyl group which may be interrupted by an ether bridge.

The dyestuffs of the Formula 1 can be obtained by coupling a tetrazo-compound of a diamine of the formula



in which  $X_1$  and  $X_2$  each represent an alkyl group which may be interrupted by an ether bridge in an alkaline medium on both sides with a 1-amino-8-hydroxynaphthalene sulfonic acid or acids, and at least on one side with a 1-amino-8-hydroxynaphthalene disulfonic acid.

The diamines of the Formula 2 used as starting materials can be obtained in known manner by the reduction of a nitro-compound of the formula



in which  $X_1$  and  $X_2$  have the meanings given above) to from a hydrazo-compound of the formula



followed by so-called benzidine rearrangement.

The compounds of the Formulae 2, 3 and 4 contain alkyl groups which are bound to the benzene nuclei through an oxygen atom and which may themselves be interrupted by an oxygen atom, that is to say, an ether bridge. Two different or identical groups of that kind may be bound to a single benzene nucleus. The groups  $X_1$  and  $X_2$  advantageously contain at most 5 carbon atoms. As examples of  $-O-X_1$  and/or  $-O-X_2$  there may be mentioned n-butoxy, n-propoxy, isopropoxy- and  $\beta$ -methoxy-ethoxy ( $O-CH_2-CH_2-O-CH_3$ ) groups but more especially ethoxy and methoxy groups. Accordingly, there may be used as diamines of the Formula 2 for making the disazodyestuffs, for example, 3:6:3':6'-tetraethoxy-4:4'-diaminodiphenyl and, advantageously, 3:6:3':6'-tetramethoxy-4:4'-diaminodiphenyl.

As coupling components for making the disazodyestuffs of the Formula 1 there are used 1-amino-8-hydroxynaphthalene sulfonic acids. The tetrazo-compounds of the diamines of the Formula 2 are coupled on at least one side with a 1-amino-8-hydroxynaphthalene disulfonic acid, and they may be coupled on the other side with a 1-amino-8-hydroxynaphthalene monosulfonic acid, such as 1-amino-8-hydroxynaphthalene-4-sulfonic acid. As examples of 1-amino-8-hydroxynaphthalene disulfonic acids there may be mentioned 1-amino-8-hydroxynaphthalene-2:4-3:5-, -3:6 and 4:6-disulfonic acid. The amino group in the 1-position may be a primary amino group or, especially in the case of the 3:6- and the 4:6-disulfonic acid, a substituted amino group, for example, a monoalkylamino



a solution containing, per liter of water, 60 grams of copper sulfate, 80 grams of potassium bromide and 15 ml. of hydrochloric acid of 30% strength.

(10) Washing in water for 5 minutes.

(11) Fixation for 5 minutes as described under 5.

(12) Washing in water for 5 minutes.

After drying, there is obtained a blue image.

The fastness to light of the image so obtained can be substantially improved by treating it for 5 to 10 minutes in a copper sulfate bath for 2 to 5% strength, or in a copper acetate bath of 2 to 4% strength, and then washing it for 5 to 10 minutes in water and drying it.

Similar blue images are obtained with the dyestuffs of the formulae

(9)



(10)



(11)



(12)



The dyestuff of the Formula 8 can be prepared as follows:

30.4 parts of 3:6:3':6'-tetramethoxy-4:4'-diamino-1:1'-diphenyl are stirred in 500 parts of water with 26 parts of hydrochloric acid of 30% strength, and dissolved, if necessary, by heating to 60° C. After the addition of a further 26 parts of hydrochloric acid, the temperature is lowered to 0° C. by the addition of ice. 14 parts of sodium nitrite, dissolved in 50 parts of water, are added in portions over a period of 10 minutes. There is formed a clear yellow solution of the tetrazo-compound. The solution so obtained is run into a solution of the coupling component, which has been prepared by dissolving 65 parts of 1-amino-8-hydroxynaphthalene-2:4-disulfonic acid and 80 parts of anhydrous sodium carbonate in 800 parts of water, and cooling the solution to 0 to 2° C. by the addition of ice. Coupling takes place rapidly. After 2 to 4 hours, the reaction mixture is heated to 65° C., and the dyestuff is precipitated by the addition of 250 to 400 parts

of sodium chloride. After cooling the mixture to 25° C., the dyestuff is isolated by filtration and dried. There are obtained about 100 parts of the dyestuff of the Formula 8.

The dyestuffs of the Formulae 9 to 12 can be prepared by the same method. For example, the dyestuff of the Formula 11 is obtained by first running the aforesaid tetrazo-compound into a solution of 32 parts of 1-amino-8-hydroxynaphthalene-2:4-disulfonic acid and 100 parts of sodium bicarbonate in 800 parts of water, and, after the formation of the diazo-azo-compound, adding a solution of 32 parts of 1-amino-8-hydroxynaphthalene-4:6-disulfonic acid and 40 parts of anhydrous sodium carbonate in 400 parts of water. After 2 hours the dyestuff is precipitated in the manner described above.

5

10

#### Example 2

200 grams of silver bromide emulsion are sensitized 50 with a red sensitizer, and mixed at 35° C. with a mixture of 0.4 gram of the dyestuff of the Formula 8, 5.0 grams of gelatine, 0.4 gram of a condensation product of dicyandiamidine with formaldehyde, and 95 cc. of water. The emulsion so obtained is cast on a suitable support.

55

#### Example 3

The procedure is the same as in Example 2, with the exception that 0.28 gram of barium chloride is added, instead of the condensation product of dicyandiamidine.

60 Stabilizers, spreading agents, such as saponin, and/or hardening agents may be incorporated with the casting solutions described in Examples 2 and 3 before they are cast.

#### Example 4

65 3 grams of the dyestuff of the formula



are dissolved in 500 ml. of water, and the solution is added to 1 liter of a red-sensitized silver bromide gelatine which contains, per liter, 30 to 35 grams of silver. 1 gram of 1:1'-diphenyl-4:4'-biguanide in the form of its acetate or hydrochloride dissolved in 100 ml. of water is added dropwise while stirring. This renders the dyestuff completely fast to diffusion. The dyestuff-gelatine emulsion so obtained is cast on a suitable support, if desired, as one of the layers of a three-color multi-layer material, and processing is carried out as described in Example 1. The developed and after-coppered blue layer possesses a high degree of fastness to light.

The dyestuff of the Formula 13 can be made as follows: 53.6 parts of 3:6:3':6' - tetra- $\beta$ -ethoxy-ethoxy-4:4'-diamino-1:1'-diphenyl are stirred for several hours in 600 parts of water in the presence of 26 parts of hydrochloric acid of 30% strength. After the addition of ice and a further 26 parts of hydrochloric acid of 30% strength, 14 parts of sodium nitrite in the form of an aqueous solution of 20% strength are added dropwise in the course of 30 minutes at a temperature of 0 to 2°C. The tetrazo-compound so obtained is stirred for 1 hour, and then added to a solution of 65 parts of 1-amino-8-hydroxy-naphthalene-2:4-disulfonic acid, 80 parts of anhydrous sodium carbonate and 40 parts of commercial picoline in 800 parts of



water. The temperature is kept at 0 to 2°C. by the addition of ice. Coupling takes place rapidly, and the dyestuff can be obtained in an easily filterable form by the addition

bleaching process which contains silver halide and a disazo-dyestuff of the formula



in which  $R_1$  and  $R_2$  each represents the radical of a 1-amino-8-hydroxynaphthalene disulfonic acid which is bound to the azo linkage in 7-position, and  $X_1$  and  $X_2$  each represents a member selected from the group consisting of an alkyl group and an alkoxyalkyl group.

10 15 2. A photographic layer suitable for the silver dyestuff bleaching process which contains silver halide and a disazo-dyestuff of the formula



20 in which  $R_1$  and  $R_2$  each represents the radical of a 1-amino-8-hydroxynaphthalene disulfonic acid which is bound to the azo linkage in 7-position.

25 3. A photographic layer suitable for the silver dyestuff bleaching process which contains silver halide and a disazo-dyestuff of the formula



4. A photographic layer suitable for the silver dyestuff bleaching process which contains silver halide and the disazo-dyestuff of the formula



of 250 parts of sodium chloride. The dyestuff is then isolated by filtration, the adherent picoline is removed by washing with aqueous alcohol, and the dyestuff is dried.

5. A photographic layer suitable for the silver dyestuff bleaching process which contains silver halide and the disazo-dyestuff of the formula



6. A photographic layer suitable for the silver dyestuff bleaching process which contains silver halide and the disazo-dyestuff of the formula



What is claimed is:

1. A photographic layer suitable for the silver dyestuff

7. A photographic layer suitable for the silver dyestuff bleaching process which contains silver halide and the disazo-dyestuff of the formula



8. A photographic layer suitable for the silver dyestuff bleaching process which contains silver halide and the disazo-dyestuff of the formula



9. A photographic layer suitable for the silver dyestuff bleaching process which contains silver halide and the disazo-dyestuff of the formula



**References Cited by the Examiner**

**UNITED STATES PATENTS**

2,304,884 12/1942 Carroll ----- 96—99  
2,612,448 9/1952 Gaspar et al. ----- 96—99

**FOREIGN PATENTS**

56,699 10/1952 France.

NORMAN G. TORCHIN, *Primary Examiner.*

J. T. BROWN, *Assistant Examiner.*